

## UNITED STATES PATENT OFFICE

ERNEST A. YOUNG AND GLENN H. ALVEY, OF SAN ANTONIO, TEXAS, ASSIGNEES TO  
UVALDE ROCK ASPHALT COMPANY, OF BEAUMONT, TEXAS, A CORPORATION OF  
TEXAS

## PAVING MATERIAL AND METHOD OF PREPARING SAME

No Drawing.

Application filed June 20, 1927. Serial No. 200,306.

This invention relates to a new and improved paving material and to a method of preparing the same, and more particularly to a material and method using a natural rock asphalt and producing a material adapted to be laid in the cold state.

In its specific form our invention relates to a method of producing a paving material having as its base a natural rock asphalt such as the Uvalde rock asphalt found in Uvalde County, Texas, although other generally similar materials may be used. This Uvalde rock asphalt consists of a comparatively porous shell limestone impregnated naturally with asphalt which thoroughly fills the pores in the rock.

The general method of using this material for paving purposes has been to crush and grade it and then to heat it and treat it with a flux such as asphaltic oil or a paraffine base oil. It is then necessary to lay and compact the material without great delay as it tends to cake and set as it cools.

Since the heating and treatment with the flux oil must take place near the work, it is necessary to set up paving mixing plants at various points and the expense of installation and maintenance of these plants adds materially to the cost of the paving.

A cold mixing process has also been developed in which the crushed rock asphalt is mixed cold with a flux, usually an asphaltic base oil. A solvent such as kerosene is also generally added to delay the setting of the mix. This mix tends to set as the volatiles in the flux and solvent evaporate and can not be transported successfully for very great distances from a paving plant. When transported the mix cakes in the cars and must be broken up with pick axes or similar tools to remove it from the cars. This adds very greatly to the expense and this method is therefore not commercially practical for producing a mix to be used at considerable distances from a paving plant.

It is an object of the present invention to provide a new and improved method of preparing a paving material or the like, and such a material which may be mixed and handled cold and may be transported before placing without serious caking of the material. 50

It is a further object of the invention to provide a method and mixture by which the natural set of the basic mixture is retarded by the addition of other elements, and in which the retardation of the set may be controlled by the amount and relation of the elements of the mixture. 55

It is an additional object to provide a paving material of this type having incorporated therein an excess of certain sizes of relatively harder material whereby the softer material is crushed and forced into intimate contact. 60

It is also an object to produce a paving material which will give a surface of a character adapted to minimize or prevent the skidding of vehicles on the surface. 65

Other and further objects will appear as the description proceeds.

The basic element in our improved paving material is the natural rock asphalt such as Uvalde asphalt which we have referred to specifically above. This consists of a relatively soft porous shell limestone impregnated with asphalt or bitumen. This asphalt forms from about eight to twelve per cent of the commercially used material. The asphaltic rock is crushed and graded according to sizes and a mixture is formed which is so proportioned as to give a minimum of voids. 70 75 80 This mixture is what is known as a balanced mix and affords a compact pavement or the like, substantially impervious to water and without air pockets.

This rock asphalt is treated with a flux which tends to soften the asphalt in the rock and cause the particles of the material to adhere to each other. If the material were used without any further addition it would cake and pack in transportation so as to make it 85 90

impractical to carry it any great distance from the mixing plant for use. In order to retard the set of the material we add to the mixture a small quantity of a solvent which may be kerosene or any other light petroleum distillate. This fluid has a solvent action both on the asphalt of the rock and upon the flux oil and retards the set of the material.

As an additional feature, when the material must be transported a considerable distance before being used or when the weather is so hot as to cause rapid evaporation, we find it desirable to add water to the mixture. A further element which we incorporate in our paving material consists in a crushed rock which is harder than the limestone rock asphalt. This crushed rock may be a rock such as trap rock or hard limestone and is preferably screened so as to eliminate the smaller particles. We have found that the most satisfactory results will be obtained by using a one-size crushed trap rock substantially the same size as the larger portions of the rock asphalt aggregate. In laying pavements of ordinary thickness, this size would be from one-fourth to one-half inch. The crushed hard rock when added to the crushed rock asphalt serves to unbalance the total mixture; that is, it will give to the total mixture a preponderance of larger aggregate so that the smaller aggregate and fine particles present will not be sufficient to fill up all voids in the mixture. This fact tends to retard the set of the material as it will cause the particles to be largely separated by air spaces. When the material is laid and compacted, however, the hard rock will be forced into the particles of rock asphalt and these particles will be further crushed so that a solid and compact pavement will result. The hard rock which extends throughout the paving gives a surface which is efficient in preventing skidding.

We have found that a very material difference may be made in the rate of set of the material, not only by varying the quantities of the several elements but also by varying the order in which the elements are mixed together. For example, the crushed rock asphalt may first have added thereto the flux and solvent mixed together. In this case the solvent is merely thinned by the flux and its action therefore retarded since it is rendered less sticky. The action will be further retarded if the solvent is first added to the rock asphalt which is thus thoroughly wetted with the solvent before the flux is applied. A still further retardation in set may be accomplished by initially dampening the rock asphalt with water before applying the solvent and flux. The wet rock asphalt will not be permeated by the flux and solvent until the water has largely evaporated as the oil will not mix with the water.

Another manner in which the materials may be mixed is by applying the flux and solvent to the crushed rock asphalt, then wetting the crushed hard rock with water and mixing the damp rock with the treated rock asphalt. The dampness of the rock prevents it from being immediately coated with the solvent and flux and serves to separate the particles of rock asphalt and to retard the set. If desired, the rock asphalt and hard rock may be mixed together and the solvent, flux and water may be added in the form of an emulsion. In some cases where long delay of set is desired, it may be found advisable to wet both the rock asphalt and rock before applying the flux and solvent, and mixing the mass together.

It will be apparent therefore that our materials may be mixed together in a variety of ways and that the method and order of mixture may be adapted to the particular needs of the temperatures present and the length of time and the distance required for transportation. These elements will preferably be so adjusted that when the material is spread out in a thin layer on the surface being covered, the volatile solvent and any water present will be sufficiently evaporated in a short time, such as a half hour, so that the material may be compacted by a heavy steam roller or the like and formed into a dense water-proof surface.

While the several elements of our mixture may be widely varied in proportion, the mixture will generally consist of from ten to thirty-three per cent of hard rock, from sixty to ninety per cent rock asphalt, and from one to three per cent flux; and, where solvent or water or both are used, from one to three per cent solvent and from one-half to two per cent or more of water.

While our material is particularly adapted for paving purposes in paving streets and roadways, it will be understood that it is also capable of many other uses. For example, it may be used to pave sidewalks or floors in buildings and may also be used in covering roofs. In view of its impermeability, it has also proved of value in covering the bottoms of reservoirs or chambers for holding liquid. The material is also efficient in dampening vibrations and is therefore particularly useful in bridge coverings, industrial flooring, railroad platforms and crossings, and engine foundations.

While we have given by way of example, certain preferred methods of mixing and preferred proportions, our invention is capable of wide modification and we contemplate such changes and modifications as come within the spirit and scope of the appended claims.

We claim:

1. The method of making a paving composition or the like which comprises crushing

rock asphalt, making up a mass of said crushed rock asphalt sized and proportioned to give a balanced mixture having a minimum of voids, treating said rock asphalt with a flux, and adding to said mixture a crushed rock which is harder than the rock asphalt and which is in sizes and quantity such as to create voids in the total mixture.

2. The method of making a paving composition or the like which comprises crushing rock asphalt, making up a mass of said crushed rock asphalt sized and proportioned to give a balanced mixture having a minimum of voids, treating said rock asphalt with a flux, and adding to said mixture a dampened crushed rock which is harder than the crushed rock asphalt and which is in size and quantity such as to create voids in the total mixture.

20 3. The method of making a paving composition or the like which comprises crushing rock asphalt, making up a mass of said crushed rock asphalt sized and proportioned to give a balanced mixture having a minimum of voids, treating said rock asphalt with a flux, and adding to said mixture a dampened crushed rock which is harder than the crushed rock asphalt and which is substantially the size of the coarser rock asphalt aggregate, said rock being so graded as to size and added in such quantity as to create voids in the whole mixture.

4. The method of making a paving composition or the like which comprises crushing rock asphalt, making up a mass of said crushed rock asphalt sized and proportioned to give a balanced mixture having a minimum of voids, treating said rock asphalt with a solvent and with a flux, and adding to said mixture a crushed rock which is harder than the crushed rock asphalt and which is substantially the size of the coarser rock asphalt aggregate, said rock being added in such quantity as to create voids in the total mixture.

45 5. The method of making a paving composition or the like which comprises crushing rock asphalt, making up a mass of said asphalt sized and proportioned to give a balanced mixture having a minimum of voids, dampening said asphalt with water, treating said asphalt with a solvent and with a flux, and mixing with the asphalt a crushed rock harder than the rock asphalt, said rock being in such sizes and quantity as to create voids in the entire mixture.

60 6. A paving mixture comprising damp crushed rock asphalt, said asphalt being sized and proportioned to a balanced mixture with a minimum of voids, a flux, and damp crushed rock harder than the crushed rock asphalt, said rock being in size and quantity such as to create voids in the entire mixture.

65 7. A paving mixture comprising crushed

rock asphalt, said asphalt being sized and proportioned to a balanced mixture with a minimum of voids, a flux, and crushed rock harder than the crushed rock asphalt, said rock being so sized and in such quantity as to produce voids in the entire mixture.

Signed at San Antonio, Texas, this 16 day of June, 1927.

ERNEST A. YOUNG.  
GLENN H. ALVEY.

75

80

85

90

95

100

105

110

115

120

125

130